

252/100

## United States Patent Office

3,442,810

Patented May 6, 1969

1

3,442,810  
CHEMICAL POLISHING COMPOSITION  
AND METHOD

Charles H. Elbreder, St. Louis, Mo., assignor to Garman Company, Incorporated, Lemay, Mo., a corporation of Missouri  
No Drawing. Filed Feb. 25, 1966, Ser. No. 529,950  
Int. Cl. C23f 3/04

U.S. CL. 252—79.4

12 Claims

## ABSTRACT OF THE DISCLOSURE

An improved aqueous polishing composition which is effective for use in polishing articles composed of copper, brass or alloys of high copper content consists of a chromium compound such as chromium trioxide or sodium chromate which provides a concentration of 2-25% by weight of chromic acid in aqueous solution, a source of elemental bromine such as sodium bromide which provides 0.05-3.5% by weight of bromine in aqueous solution and either sulfamic acid or sulfuric acid in an amount sufficient to provide a pH of 0.1 to 2.0. The composition may be prepared in dry form and then dissolved in water to form an aqueous polishing composition. The copper article is contacted with the aqueous composition for a brief period and the reddish brown film which forms thereon is then removed by dipping the article in an acid or alkaline medium or by heating the article to a temperature above 180° F. The resulting article displays a smooth, bright finish having a high degree of luster.

The invention relates to chemical polishing and more particularly to compositions and methods for chemically polishing articles composed of copper, brass or alloys of high copper content.

Briefly, the present invention is directed to a dry composition soluble in water to form an aqueous polishing composition for use in polishing articles composed of copper, brass or alloys of high copper content comprising a chromium compound which is converted into chromic acid upon being dissolved in acidified water, an alkali metal bromide and sulfamic acid. The invention is also directed to aqueous polishing compositions formed by dissolving dry compositions of the above type in water and to methods of chemical polishing utilizing such aqueous compositions.

Among the several objects of the invention may be noted the provision of improved compositions for use in polishing articles composed of copper, brass or alloys of high copper content; the provision of such compositions which impart to copper articles a smooth, bright finish having a high degree of luster; the provision of compositions of this type which simultaneously achieves removal of coarse projections and dissolving of smaller surface irregularities from the surface of the treated articles; and the provision of methods of chemically polishing copper articles with compositions of the type mentioned which may be conveniently carried out and which give reliable results. Other objects and features will be in part apparent and in part pointed out hereinafter.

The invention accordingly comprises the products and methods hereinafter described, the scope of the invention being indicated in the following claims.

As is known, chemical polishing or brightening compositions have been formulated and used heretofore for the purpose of polishing and imparting a brightened surface to articles such as fittings, for example, composed of copper, brass or alloys of high copper content. However, such compositions have not proved entirely satisfactory

2

in practice and have suffered from certain shortcomings in that they do not impart a uniformly bright surface to copper and brass articles, and also, do not produce a smooth, level surface substantially free of projections and other surface irregularities. Upon examination, it is seen that the surface of copper and brass articles to be polished is consistently irregular in profile. These irregularities consist of projections and depressions or peaks and valleys on the surface.

5 A high degree of smoothness and brightness of the surface of copper articles is desirable particularly where such articles are to be nickel plated. When the surface of a copper or brass article is smooth and contains no surface irregularities, considerably less nickel is required to obtain a high luster for the plated article. There remains, therefore, an unfulfilled need for an improved polishing composition which does not exhibit the aforementioned drawbacks.

10 In accordance with the present invention, it has now been found that improved results in the chemical polishing of copper and brass articles may be achieved through the use of a composition containing a chromium compound which is converted into chromic acid upon being dissolved in acidified water, an alkali metal bromide and sulfamic acid. Upon being dissolved in water, such a composition provides an improved aqueous polishing composition for chemically polishing articles composed of copper, brass or alloys of high copper content. I have found that the polishing compositions of my invention 15 simultaneously effect macropolishing (i.e., the removal of coarse projections from and leveling of the surface) and micropolishing (i.e., the dissolving of smaller surface irregularities and polishing of the surface), and thereby 20 impart smoothness and brightness, respectively, to the surface of the copper article.

25 It is believed that the presence of elemental bromine and chromic acid in an aqueous solution having a low pH value is responsible for imparting unique leveling and chemical polishing characteristics to the surface of 30 the article treated therewith. The elemental bromine is provided by adding elemental bromine per se to the aqueous solution or by incorporating an alkali metal bromide in the dry composition which is added to water to form my aqueous polishing composition. The alkali metal bromides, such as sodium and potassium bromides, are oxidized and release free bromine in an aqueous solution having a low pH.

35 The chromic acid in the aqueous composition is provided by incorporating in the dry composition a chromium compound which is converted into chromic acid upon being dissolved in acidified water. Preferably, chromium trioxide is employed as the chromium compound as this is readily converted into chromic acid upon being dissolved in water. However, it will be understood that 40 alkali metal chromates such as sodium chromate and potassium chromate and alkali metal dichromates such as sodium dichromate and potassium dichromate, may also be employed to provide chromic acid in the aqueous polishing composition of my invention.

45 In order to provide the low pH for the aqueous composition containing the chromic acid and elemental bromine, either sulfamic acid or sulfuric acid may be included. Sulfamic acid is preferred since it has been found to give a somewhat better surface finish to the copper article being treated. Moreover, being a solid, sulfamic acid may be incorporated in the dry composition described above.

50 In the practice of the invention, it has been found that the amount of free bromine present in aqueous solution with chromic acid and sulfamic or sulfuric acid should be between approximately 0.05% and 3.5% by weight in order to achieve enhanced chemical polishing

of copper and brass articles. For good results, the aqueous solution should contain between approximately 2% and 25% by weight of chromic acid. Further, the solution should contain a sufficient amount of sulfamic acid or sulfuric acid to give the solution a pH between approximately 0.1 and 2.0.

For convenience, I prefer to employ a dry composition as described above in carrying out the invention since it is merely necessary to dissolve the dry composition in an appropriate quantity of water to obtain an aqueous polishing composition. However, if desired, the aqueous polishing composition may be prepared by dissolving the individual components in the necessary amount of water. In the latter case, of course, it is possible to use elemental bromine as the source of bromine and sulfuric acid to provide a low pH whereas these particular components may not be incorporated in the dry composition.

In carrying out the invention, a dry composition containing a chromium compound convertible into chromic acid upon being dissolved in acidified water, an alkali metal bromide and sulfamic acid is first dissolved in water to provide an aqueous solution having a pH within the limits stated above and containing chromic acid and free bromine. Alternatively, such an aqueous solution may be formed by dissolving chromium trioxide or an alkali metal chromate or dichromate in water together with elemental bromine or an alkali metal bromide and either sulfamic or sulfuric acid. In either event, the amount of components employed should be within the ranges hereinbefore stated. The copper or brass article to be treated is then immersed in the aqueous solution for a relatively short period of time which may range from a few seconds to about five minutes. Immediately after immersion, it will be observed that a reddish brown film is formed on the surface of the metal article. After the desired immersion period the article or metal part is removed from the aqueous solution and preferably rinsed in water to wash away the aqueous polishing solution remaining thereon.

Next, the reddish brown film is removed and this is preferably effected by dipping the article in an alkaline or acid medium. It has been found that the reddish brown film formed on the surface of the copper article is insoluble in cold water and only slightly soluble in hot water. However, the film is readily soluble in alkaline and acid media. Any of the conventional acid or alkaline media may be used. For example, a solution containing between 2% and 10% by weight of sodium hydroxide or one containing between 2% and 10% by weight of sulfuric acid or sulfamic acid has been found satisfactory for this purpose.

If desired, the reddish brown film may be removed by heating the article to a temperature of at least 180° F., preferably a temperature between 180° F., and 200° F.

Following removal of the film, the article may be given a final water rinse to wash away traces of the acid or alkaline media used in removing the film. The surface of the article thus produced through the practice of the invention exhibits a high degree of luster and polish and is substantially smooth and free of projections and irregularities.

Although the exact nature of the reddish brown film formed on the surface of the article is not known, it is believed the film consists of a cupric chromate complex compound having the formula  $CuCrO_4 \cdot 2CuO \cdot 2H_2O$ . This film is somewhat gelatinous in nature and forms uniformly over the entire surface being treated. It is believed that the metal being treated becomes anodic upon being submerged in the above described aqueous solution and that the film is responsible for micropolishing of the surface by chemical oxidation. The film apparently allows the necessary exchange of electrons between the metal being polished and the ions in solution. In any event, the resulting surface is smooth and bright.

The following examples illustrate the invention.

#### Example 1

An aqueous solution was prepared containing 10% by weight of chromium trioxide and 10% by weight of sulfamic acid. Upon being dissolved in water, the chromium trioxide was converted into chromic acid. The solution had a pH of 0.5. To the solution was added 0.2% by weight of elemental bromide. A copper fitting was immersed in the resulting solution whereupon a reddish brown film immediately formed on the surface thereof. After three minutes, the fitting was removed from the solution and rinsed in water. The fitting was next dipped in a 2% sodium hydroxide solution to remove the reddish brown film. The fitting was then given a final water rinse. The resulting fitting exhibited a high degree of luster, brightness and smoothness.

#### Example 2

A dry composition soluble in water to form an aqueous polishing composition for use in polishing articles composed of copper, brass or alloys of high copper content, was prepared having the following composition by weight—

| Component:        | Percentage by weight |
|-------------------|----------------------|
| Chromium trioxide | 53.8                 |
| Sulfamic acid     | 44.8                 |
| Potassium bromide | 1.4                  |
|                   | 100.0                |

#### Example 3

The composition of Example 2 was dissolved in water to form the following aqueous polishing composition—

| Component:        | Percentage by weight |
|-------------------|----------------------|
| Chromium trioxide | 12.0                 |
| Sulfamic acid     | 10.0                 |
| Potassium bromide | 0.3                  |
| Water             | 77.7                 |
|                   | 100.0                |

This aqueous polishing composition was used as described in Example 1 to polish a copper article with good results.

#### Example 4

An aqueous polishing composition was prepared having the following composition by weight—

| Component:        | Percentage by weight |
|-------------------|----------------------|
| Chromium trioxide | 18.0                 |
| Sulfuric acid     | 5.0                  |
| Bromine           | 0.3                  |
| Water             | 76.7                 |
|                   | 100.0                |

The composition was prepared by dissolving the chromium trioxide, sulfuric acid and bromine in water. The composition was used as described in Example 1 with good results.

#### Example 5

A dry composition was prepared having the following composition by weight—

| Component:        | Percentage by weight |
|-------------------|----------------------|
| Sodium dichromate | 52.6                 |
| Sulfamic acid     | 42.1                 |
| Potassium bromide | 5.3                  |
|                   | 100.0                |

## Example 6

The composition of Example 5 was dissolved in water to form the following aqueous polishing composition—

| Component:        | Percentage by weight |
|-------------------|----------------------|
| Sodium dichromate | 15.0                 |
| Sulfamic acid     | 12.0                 |
| Potassium bromide | 1.5                  |
| Water             | 71.5                 |
|                   | 100.0                |

The resulting aqueous polishing composition was used as described in Example 1 with good results.

## Example 7

An aqueous polishing composition was prepared having the following composition by weight—

| Component:        | Percentage by weight |
|-------------------|----------------------|
| Chromium trioxide | 8.0                  |
| Sulfamic acid     | 8.0                  |
| Bromine           | 0.1                  |
| Water             | 83.9                 |
|                   | 100.0                |

The composition was prepared and used as described in Example 1 with good results.

## Example 8

A dry composition was prepared having the following composition by weight—

| Component:        | Percentage by weight |
|-------------------|----------------------|
| Chromium trioxide | 56.7                 |
| Sulfamic acid     | 39.0                 |
| Sodium bromide    | 4.3                  |
|                   | 100.0                |

## Example 9

The composition of Example 8 was dissolved in water to form the following aqueous polishing composition—

| Component:        | Percentage by weight |
|-------------------|----------------------|
| Chromium trioxide | 15.0                 |
| Sulfamic acid     | 11.0                 |
| Sodium bromide    | 2.2                  |
| Water             | 71.8                 |
|                   | 100.0                |

The resulting aqueous polishing composition was used as described in Example 1 with good results.

In view of the above, it will be seen that the several objects of the invention are achieved and other advantageous results attained.

As various changes could be made in the above methods and products without departing from the scope of the invention, it is intended that all matter contained in the above description shall be interpreted as illustrative and not in a limiting sense.

What is claimed is:

1. A dry composition soluble in water to form an aqueous polishing composition for use in polishing articles composed of copper, brass or alloys of high copper content consisting essentially of a chromium compound selected from the group consisting of chromium trioxide, alkali metal chromates and alkali metal dichromates, an alkali metal bromide and sulfamic acid, the amount of said chromium compound in the composition providing a concentration of between 2% and 25% by weight of chromic acid in aqueous solution, the amount of said

alkali metal bromide in the composition providing between 0.05% and 3.5% by weight of bromine in aqueous solution and the amount of sulfamic acid in the composition being sufficient to provide a pH of approximately 0.1 to 2.0 for the aqueous solution formed by dissolving the composition in water.

2. A dry composition as set forth in claim 1 in which the chromium compound is chromium trioxide and the alkali metal bromide is potassium bromide.

3. A dry composition as set forth in claim 1 wherein the chromium compound is sodium dichromate.

4. An aqueous polishing composition for use in polishing articles composed of copper, brass or alloys of high copper content consisting essentially of water, a chromium compound selected from the group consisting of chromium trioxide, chromic acid, alkali metal chromates and alkali metal dichromates, a source of bromine selected from the group consisting of elemental bromine and alkali metal bromides and an acid selected from the group consisting of sulfamic acid and sulfuric acid, the amount of said chromium compound in the composition providing a concentration of between 2% and 25% by weight of chromic acid in aqueous solution, the amount of said source of bromine in the composition providing between 0.05% and 3.5% by weight of bromine in aqueous solution and the amount of said acid in the composition being sufficient to provide a pH of approximately 0.1 to 2.0 for the composition.

5. An aqueous polishing composition as set forth in claim 4 wherein the chromium compound is chromic acid, the source of bromine is elemental bromine and the acid is sulfamic acid.

6. An aqueous polishing composition as set forth in claim 4 wherein the chromium compound is chromium trioxide and the alkali metal bromide is potassium bromide.

7. An aqueous polishing composition as set forth in claim 4 wherein the chromium compound is sodium dichromate.

8. The method of chemically polishing an article composed of copper, brass or alloys of high copper content to impart a smooth, bright finish having a high degree of luster which comprises the steps of contacting said article with an aqueous polishing composition consisting essentially of water, a chromium compound selected from the group consisting of chromium trioxide, chromic acid, alkali metal chromates and alkali metal dichromates, a source of bromine selected from the group consisting of elemental bromine and alkali metal bromides and an acid selected from the group consisting of sulfamic acid and sulfuric acid, the amount of said chromium compound in the composition providing a concentration of between 2% and 25% by weight of chromic acid in aqueous solution, the amount of said source of bromine in the composition providing between 0.05% and 3.5% by weight of bromine in aqueous solution and the amount of said acid in the composition being sufficient to provide a pH of approximately 0.1 to 2.0 for the composition, and thereafter removing the film formed on said article by subjecting the article to treatment with an alkaline or acid medium or by heating the article to a temperature of about 180 to 200° F.

9. The method of chemically polishing as set forth in claim 8 wherein the chromium compound is chromic acid, the source of bromine is elemental bromine and the acid is sulfamic acid.

10. The method of chemically polishing as set forth in claim 8 wherein the article is given a water rinse before and after removal of said film therefrom.

11. The method of chemically polishing as set forth in claim 8 wherein the alkaline medium is sodium hydroxide.

12. The method of chemically polishing as set forth in claim 8 wherein the acid medium is sulfamic acid.

## References Cited

## UNITED STATES PATENTS

3,081,211 3/1963 Rich et al. ----- 212—79.2 XR  
 3,248,235 4/1966 Pryor et al. ----- 106—3  
 3,249,523 5/1966 Post et al. ----- 212—79.2 XR  
 3,269,881 8/1966 Alderuccio et al. --- 156—18 XR  
 3,272,748 9/1966 Szkudlapski ----- 212—79.3

3,274,114 9/1966 Grof ----- 252—100  
 3,290,174 12/1966 Kendall ----- 156—18 XR  
 3,322,673 5/1967 Slominski ----- 212—79.1 XR

5 MAYER WEINBLATT, *Primary Examiner.*

U.S. CL. X.R.

134—27; 156—14, 17, 18; 252—79.1, 79.2, 100, 142